

Feb. 3, 1959

W. G. LEE

2,872,354

PROCESSES OF CONTINUOUS CHEMICAL NICKEL PLATING

Original Filed Dec. 31, 1954



BY

Smith, Olsen, Baird & Miller,  
Attns.

INVENTOR.

WARREN G. LEE

2,872,354

## PROCESSES OF CONTINUOUS CHEMICAL NICKEL PLATING

Warren G. Lee, East Chicago, Ind., assignor to General American Transportation Corporation, Chicago, Ill., a corporation of New York

Original application December 31, 1954, Serial No. 479,040. Divided and this application March 26, 1956, Serial No. 573,789.

7 Claims. (Cl. 117—130)

The present invention relates to processes of continuous nickel plating of catalytic materials; and it is the general object of the invention to provide an improved process of the general character of that disclosed in U. S. Patent No. 2,717,218, granted on September 6, 1955, to Paul Talmey and William J. Crehan. This application is a division of the copending application of Paul Talmey, Gregoire Gutzeit and Donald E. Metheny, Serial No. 479,040, filed December 31, 1954, now abandoned, which application was originally filed, through error and without any deceptive intention, jointly by: Paul Talmey, Gregoire Gutzeit, Donald E. Metheny and Warren G. Lee.

The chemical nickel plating of a catalytic material employing an aqueous bath of the nickel cation-hypophosphite anion type is based upon the catalytic reduction of nickel cations to metallic nickel and the corresponding oxidation of hypophosphite anions to phosphite anions with the evolution of hydrogen gas at the catalytic surface. The reactions take place when the body of catalytic material is immersed in the plating bath, and the exterior surface of the body of catalytic material is coated with nickel. The following elements are catalytic for the oxidation of hypophosphite anions and thus may be directly nickel plated: iron, cobalt, nickel, ruthenium, rhodium, palladium, osmium, iridium and platinum. The following elements are examples of materials which may be nickel plated by virtue of an initial displacement deposition of nickel thereon either directly or through a galvanic effect: copper, silver, gold, beryllium, germanium, aluminum, carbon, vanadium, molybdenum, tungsten, chromium, selenium, titanium and uranium. The following elements are examples of non-catalytic materials which ordinarily may not be nickel plated: bismuth, cadmium, tin, lead and zinc. The activity of the catalytic materials varies considerably and the following elements are particularly good catalysts in the chemical nickel plating bath: iron, cobalt, nickel and palladium. The chemical nickel plating process is autocatalytic since both the original surface of the body being plated and the nickel metal that is deposited on the surface thereof are catalytic. As time proceeds, the anions, as contrasted with the cations of the nickel salt that is dissolved in the plating bath, combine with the hydrogen cations to form an acid, which, in turn, lowers the pH of the plating bath.

In the continuous plating process disclosed in the Talmey and Crehan patent, the plating bath is regenerated continuously by the addition thereto of soluble nickel-containing and hypophosphite-containing reagents, as well as an alkalizing reagent for pH control; which regeneration of the plating bath during the plating of the catalytic material maintains not only the desired nickel cation concentration and hypophosphite anion concentration, but also preserves the most advantageous pH of the plating bath to assure a high plating rate. The continuous nickel plating process and system disclosed in this patent involves a plating chamber and a reservoir; and in the arrangement the plating solution is circulated from the reservoir to the plating chamber and back to the reservoir, the plating solution being heated to a relatively high temperature slightly below the boiling point thereof after withdrawal from the reservoir and before introduction into the plating chamber, and the plating solution being cooled to a relatively low temperature well below the boiling point thereof after withdrawal from the plating chamber and before return into the reservoir. Of course, the catalytic body or bodies are plated by immersion in the plating solution in the plating chamber, while the plating solution is regenerated in the reservoir by the addition of the previously mentioned reagents thereto in the reservoir.

10 The catalytic body is subsequently withdrawn from the plating solution in the plating chamber after a time interval corresponding to the thickness of the nickel plating thereon that is desired.

A number of suitable aqueous chemical nickel plating 15 baths of the nickel cation-hypophosphite anion type that may be employed in the continuous nickel plating system of the Talmey and Crehan patent are disclosed in U. S. Patent No. 2,658,841, granted on November 10, 1953, to Gregoire Gutzeit and Abraham Krieg and in U. S. Patent No. 2,658,842, granted on November 10, 1953, to Gregoire Gutzeit and Ernest J. Ramirez and in the copending applications of Gregoire Gutzeit, Paul Talmey and Warren G. Lee, Serial No. 478,492, filed December 29, 1954; Serial No. 479,088, filed December 31, 1954, now Patent 25 No. 2,822,293, and Serial No. 569,815, filed March 6, 1956, now Patent No. 2,822,294. A plating bath of these types fundamentally comprises an aqueous solution of nickel ions and hypophosphite ions; and such a bath may comprise an absolute concentration of hypophosphite ions 30 in the range 0.15 to 1.20 moles/liter, a ratio between nickel ions and hypophosphite ions in the range 0.25 to 1.60, and an initial pH in the approximate range 4 to 7. In the continuous plating system, the plating baths disclosed in the Gutzeit, Talmey and Lee applications are preferred, 35 both from the standpoint of economy and of performance; a preferred bath of this type essentially comprises an aqueous solution of nickel ions and hypophosphite ions and lactic ions and propionic ions, the absolute concentration of hypophosphite ions being in the range 0.15 to 40 1.20 moles/liter, the ratio between nickel ions and hypophosphite ions being in the range 0.25 to 1.60, the absolute concentration of lactic ions being in the range 0.25 to 0.60 mole/liter, the absolute concentration of propionic ions being in the range 0.025 to 0.060 mole/liter, and the bath having an initial pH in the range 4.4 to 5.6; and 45 four typical examples of such aqueous plating baths are as follows:

## Bath I

|                                                        |                               |
|--------------------------------------------------------|-------------------------------|
| Nickel ions (as nickel sulfate) ---                    | 0.08 m. p. l.                 |
| Hypophosphite ions (as sodium hy-<br>poposphite) ----- | 0.230 m. p. l.                |
| Lactic acid -----                                      | 0.30 to 0.40 m. p. l.         |
| Lead sulfide (stabilizer) -----                        | 1 p. p. m. Pb <sup>++</sup> . |
| pH adjusted to 4.6 with NaOH.                          |                               |

## Bath II

|                                                        |                               |
|--------------------------------------------------------|-------------------------------|
| Nickel ions (as nickel sulfate) -----                  | 0.07 to 0.08 m. p. l.         |
| Hypophosphite ions (as sodium hy-<br>poposphite) ----- | 0.225 m. p. l.                |
| Lactic acid -----                                      | 0.30 to 0.40 m. p. l.         |
| Propionic acid -----                                   | 0.03 m. p. l.                 |
| Lead sulfide (stabilizer) -----                        | 1 p. p. m. Pb <sup>++</sup> . |
| pH adjusted to 4.6 with NaOH.                          |                               |

## Bath III

|                                                         |                               |
|---------------------------------------------------------|-------------------------------|
| Nickel ions (as nickel sulfate) -----                   | 0.08 m. p. l.                 |
| Hypophosphite ions (as sodium hypo-<br>phosphite) ----- | 0.225 m. p. l.                |
| Lactic acid -----                                       | 0.20 m. p. l.                 |
| Succinic acid -----                                     | 0.06 m. p. l.                 |
| Lead sulfide (stabilizer) -----                         | 1 p. p. m. Pb <sup>++</sup> . |
| pH adjusted to 4.6 with NaOH.                           |                               |

## Bath IV

|                                                    |                               |
|----------------------------------------------------|-------------------------------|
| Nickel ions (as nickel sulfate) .....              | 0.07 m. p. l.                 |
| Hypophosphite ions (as sodium hypophosphite) ..... | 0.230 m. p. l.                |
| Malic acid .....                                   | 0.06 m. p. l.                 |
| Lactic acid .....                                  | 0.20 m. p. l.                 |
| Succinic acid .....                                | 0.20 m. p. l.                 |
| Lead sulfide (stabilizer) .....                    | 1 p. p. m. Pb <sup>++</sup> . |
| pH adjusted to 4.6 with NaOH.                      |                               |

In addition, each of the Baths I, II, III and IV contains a high-temperature stable, chemically inert, wetting agent of any suitable type; and in these baths the function of the organic additives (malic acid, lactic acid, succinic acid and propionic acid) is three-fold, as they act as: (1) buffers; (2) exaltants (plating rate "boosters"); (3) complexing agents (to prevent precipitation of nickel phosphite at high concentrations of HPO<sub>3</sub><sup>2-</sup> ions).

Of these organic additives, lactic acid combines the three effects named, succinic and propionic acids function principally as exaltants, while malic acid functions mainly as a complexing agent.

In the formulation of any one of these plating baths, an aqueous solution is prepared of the ingredients named; the nickel cations may be derived from nickel sulfate, nickel chloride, etc., or various combinations thereof; the hypophosphite anions may be derived from sodium hypophosphite, potassium hypophosphite, etc., or various combinations thereof; the other additives are introduced into the bath normally as the acids, or as the soluble salts thereof, etc.; and the desired pH of the bath is established by the eventual introduction thereinto of an acid or a base, as required, sulfuric acid and sodium hydroxide being recommended as a matter of economy and simplicity.

In the compositions of the various plating baths, the terms "cation," "anion" and "ion," as employed, include the total quantity of the corresponding elements that are present in the plating bath, i. e., both the undisassociated and dissociated material. In other words, 100% dissociation is assumed when the terms noted are used in connection with molar ratios and concentrations in the plating bath.

In the operation of the continuous plating system disclosed in the Talmey and Crehan patent, the whole body of plating solution, as a matter of volume, is continuously circulated from the reservoir to the plating chamber and back to the reservoir to constitute what may be termed a "cycle" of circulation; and continuous regeneration thereof is accomplished in the reservoir by the continuous introduction thereinto of the reagents previously mentioned. Now after the whole body of plating solution has been used in production plating in a plurality of cycles of circulation, with the required regeneration thereof, its content in phosphite anions builds-up to a point where even the presence of relatively large quantities of complexing agents (necessarily rather weak complexing agents) cannot prevent the precipitation of nickel phosphite therein. This point is reached when the phosphite concentration attains 0.7 to 1.5 m. p. l., depending on the particular bath composition. The nickel phosphite precipitate in the plating solution forms a suspensoid whose semi-colloidal particles causes roughness of the plating on the catalytic bodies undergoing the plating operation, and also act as nuclei for thermal catalytic decomposition of the whole body of plating solution, i. e., the formation of "black precipitate" therethrough. When this point is reached, the whole body of plating solution may be termed "depleted" and has to be replaced with a freshly prepared body of plating solution in order to continue satisfactory plating of the catalytic bodies in the plating chamber.

A depleted plating bath may have, for instance, the following approximate composition:

|                          | M. p. l.  |
|--------------------------|-----------|
| Nickel ions .....        | 0.07-0.08 |
| Hypophosphite ions ..... | 0.22-0.24 |
| Phosphite ions .....     | 0.70-1.50 |
| Sulfate ions .....       | 0.65-0.70 |
| Lactic ions .....        | 0.20-0.40 |
| Sodium ions .....        | q.s.      |

Typical examples of a few depleted plating baths of the type previously described were found to have the following compositions:

|                                        | Depleted bath IA | M. p. l. |
|----------------------------------------|------------------|----------|
| Ni ions .....                          | 0.07             |          |
| NaH <sub>2</sub> PO <sub>2</sub> ..... | 0.22             |          |
| Na <sub>2</sub> HPO <sub>3</sub> ..... | 0.80             |          |
| Lactic acid .....                      | 0.30             |          |

|                                        | Depleted bath IIA | 0.07 |
|----------------------------------------|-------------------|------|
| Ni ions .....                          | 0.22              |      |
| NaH <sub>2</sub> PO <sub>2</sub> ..... | 0.80              |      |
| Na <sub>2</sub> HPO <sub>3</sub> ..... | 0.30              |      |
| Propionic acid .....                   | 0.03              |      |

|                                        | Depleted bath IIIA | 0.084 |
|----------------------------------------|--------------------|-------|
| Ni ions .....                          | 0.201              |       |
| NaH <sub>2</sub> PO <sub>2</sub> ..... | 0.671              |       |
| Na <sub>2</sub> HPO <sub>3</sub> ..... | 0.20               |       |
| Succinic acid .....                    | 0.06               |       |

|                                        | Depleted bath IVA | 0.068 |
|----------------------------------------|-------------------|-------|
| Ni ions .....                          | 0.225             |       |
| NaH <sub>2</sub> PO <sub>2</sub> ..... | 0.74              |       |
| Na <sub>2</sub> HPO <sub>3</sub> ..... | 0.06              |       |
| Malic acid .....                       | 0.2025            |       |
| Lactic acid .....                      | 0.20              |       |
| Succinic acid .....                    |                   |       |

|                                        | Depleted bath IVB | 0.07 |
|----------------------------------------|-------------------|------|
| Ni ions .....                          | 0.20              |      |
| NaH <sub>2</sub> PO <sub>2</sub> ..... | 0.86              |      |
| Na <sub>2</sub> HPO <sub>3</sub> ..... | 0.06              |      |
| Malic acid .....                       | 0.20              |      |
| Lactic acid .....                      |                   |      |
| Succinic acid .....                    |                   |      |

While the regeneration of the plating solution in the continuous plating process as disclosed in the Talmey and Crehan patent, and involving the continuous addition thereto of the reagents mentioned, contributes very substantially to economical industrial plating operation, it is apparent that this regeneration of the plating solution does not proceed as far as is desirable in order to achieve maximum economy, since it will be observed from the compositions of the foregoing depleted plating baths that there are substantial values therein that might be further utilized.

Accordingly, it is another object of the invention to provide a continuous chemical nickel plating process of the character described that involves regeneration of the plating baths, not only by the addition thereto of nickel-containing and hypophosphite-containing and alkalizing reagents, but also by the removal therefrom of phosphite ions, whereby depleted plating baths may be restored for further use.

A further object of the invention is to provide an improved process of restoring a depleted chemical nickel plating bath so that it may be employed for further use in the plating of catalytic bodies, which involves not only the removal of phosphite ions therefrom, but also the removal of other ions that have been built-up therein

as a consequence of the additions thereto of the reagents named.

A still further object of the invention is to provide an improved process of restoring a depleted chemical nickel plating bath so that it may be employed for further use in the plating of catalytic bodies, which does not introduce any substantial foreign ions thereinto and which effects the recovery of the valuable nickel cations, hypophosphite anions and organic additives therein.

The present invention is predicated upon the discovery that a depleted chemical nickel plating bath may be restored for further satisfactory use in a continuous chemical nickel plating system of the character described, by proper treatment of the depleted plating bath to remove therefrom phosphite anions and other ions that have been built-up therein by the addition of the make-up reagents, without the introduction of foreign ions, so that the resulting aqueous solution fundamentally containing nickel cations, hypophosphite anions and organic additives may then be directly restored merely by adding thereto nickel-containing hypophosphite-containing and acidifying or alkalizing reagents.

Still further features of the invention pertain to the particular arrangement of the steps of the process, whereby the above-outlined and additional operating features thereof are attained.

The invention, both as to its organization and principle of operation, together with further objects and advantages thereof, will best be understood by reference to the following specification taken in connection with the accompanying drawing, in which the single figure is a diagrammatic illustration of a continuous nickel plating system in which the process of the present invention may be carried out.

Referring now to the drawing, the continuous chemical nickel plating system there illustrated, and suitable for the carrying out of the present process, is essentially of the arrangement disclosed in the Talmey and Crehan patent. More particularly, the system fundamentally comprises a first reservoir 11a, a second reservoir 11b, a plating tank or chamber 12, a condenser 13, a primary vacuum flash tank 14, a secondary vacuum flash tank 15, a primary steam jet pump 16, a secondary steam jet pump 17, and a mechanical pump 18. The reservoir 11a includes a baffled storage compartment 19a and a communicating regeneration compartment 20a; while the reservoir 11b includes a baffled storage compartment 19b and a communicating regeneration compartment 20b. In the arrangement, the inlet of the pump 18 selectively communicates with the upper and lower portions of the storage compartments 19a and 19b via respectively associated control valves 21a-22a and 21b-22b; and the outlet of the pump 18 communicates with the upper portion of the condenser 13. The lower portion of the condenser 13 communicates with the upper portion of the plating tank 12; and the lower portion of the plating tank 12 communicates with the upper portion of the primary vacuum flash tank 14. The lower portion of the primary vacuum flash tank 14 communicates with the upper portion of the secondary vacuum flash tank 16; and the lower portion of the secondary vacuum flash tank 15 selectively communicates with the upper portions of the regeneration compartments 20a and 20b via respectively associated control valves 23a and 23b. Also, the upper portion of the primary vacuum flash tank 14 communicates with the primary steam jet pump 16, that is also connected to an associated source of high-pressure steam, not shown; and the discharge from the primary steam jet pump 16 communicates with the upper portion of the condenser 13. Also, the upper portion of the secondary vacuum flash tank 15 communicates with the secondary steam jet pump 17, that is also connected to the associated source of high-pressure steam, not shown; and the discharge from the secondary steam jet pump 17 communicates with the atmosphere. This system con-

tains an aqueous chemical plating solution of the character previously described; whereby a first portion of the plating solution is stored in one of the reservoirs 11a or 11b at a relatively low temperature well below the boiling point thereof and in a relatively concentrated form; while a second portion of the plating solution is held as a bath in the plating tank or chamber 12 at a relatively high temperature slightly below the boiling point thereof and in a relatively dilute form.

In the operation of the system, the plating solution in the storage compartment 19a or 19b may have a temperature of about 150° F.; while the plating solution in the plating tank 12 may have a temperature of about 210° F. The plating solution is circulated from the upper portion of the storage compartment 19a or 19b (depending upon which of the control valves 21a or 21b occupies its open position) by the pump 18 into the upper portion of the condenser 13, wherein it is both heated to the required temperature of about 210° F. and diluted to the required concentration by the discharge from the primary steam jet pump 16. The dilution of the plating solution in the condenser 13 is achieved not only by the introduction of the steam thereinto, but also by the introduction of the water vapor thereinto that is withdrawn from the upper portion of the primary vacuum flash tank 14 by the primary steam jet pump 16. The plating solution from the condenser 13 is circulated into the plating tank 12 and thence into the upper portion of the primary vacuum flash tank 14 and therefrom into the upper portion of the secondary vacuum flash tank 15, and ultimately back into the upper portion of the regeneration compartment 20a or 20b (depending upon which of the control valves 23a or 23b occupies its open position). In the primary vacuum flash tank 14, a vacuum of about 12" Hg is drawn by the primary steam jet pump 16; whereby water vapor is withdrawn from the contained plating solution, as previously noted, so that the plating solution in the primary vacuum flash tank 14 is both concentrated and cooled prior to introduction into the secondary vacuum flash tank 15. In the secondary vacuum flash tank 15, a vacuum of about 22" Hg is drawn by the secondary steam jet pump 17; whereby water vapor is withdrawn from the contained plating solution, so that the plating solution in the secondary vacuum flash tank 15 is both further concentrated and cooled prior to the return thereof to the regeneration compartment 20a or 20b. The plating solution returned into the regeneration compartment 20a or 20b may have a temperature of about 150° F., as previously noted, as a consequence of the tandem cooling effects produced in the primary vacuum flash tank 14 and in the secondary vacuum flash tank 15. Also, the plating solution thus returned to the regeneration compartment 20a or 20b is in the relatively concentrated form, as previously noted, as a consequence of the tandem concentrating effects produced in the primary vacuum flash tank 14 and in the secondary vacuum flash tank 15. Since the discharge of the secondary steam jet pump 17 is to the atmosphere, the water vapor withdrawn from the plating solution in the upper portion of the secondary vacuum flash tank 15 prevents the build-up of water in the circulated plating solution; and preferably, the weight of the steam introduced into the plating solution in the condenser 13 by the primary steam jet pump 16 substantially equals the weight of the water vapor withdrawn therefrom in the secondary vacuum flash tank 15 and discharged to the atmosphere by the secondary steam jet pump 17, thereby maintaining the desired balance of the weight of water supplied to and the weight of water extracted from the circulated plating solution.

The catalytic bodies are immersed in the plating bath in the plating chamber 12, whereby the metallic nickel (actually an alloy of nickel and phosphorus having a composition of about 89% to 97% nickel and 11% to 3% phosphorus by weight) is deposited upon the surfaces

thereof; and the bodies are withdrawn from the plating bath when the coatings thereon are of the desired thickness. Incident to the plating of the nickel upon the catalytic bodies, the initial composition of the plating bath is altered by the reduction of the nickel cations and the oxidation of the hypophosphite anions, as previously noted, and the initial pH of the bath is reduced, as previously explained; whereby it is necessary to regenerate the plating solution in the regeneration compartment 20a or 20b by the addition thereto of an alkalizing reagent to restore the initial pH thereof and of a soluble nickel salt and a soluble hypophosphite to restore the initial composition thereof with respect to nickel cations and hypophosphite anions, the reagents mentioned being supplied into the regeneration compartment 20a or 20b, and being thoroughly dissolved and mixed therewith before circulation back into the communicating storage compartment 19a or 19b.

Further, the system comprises make-up equipment 30 that may include five tanks 31 to 35, inclusive, that selectively communicate with make-up conduits 36 and 37 communicating with the regeneration compartments 20a and 20b. More particularly, the tanks 31 to 35, inclusive, may be selectively connected to the conduit 36 via respective control valves 41 to 45, inclusive, and the tanks 31 to 35, inclusive, may be selectively connected to the conduit 37 via respective control valves 51 to 55, inclusive. As a matter of convenience, the added alkalizing reagent may be derived from an aqueous sodium hydroxide stock solution stored in the tank 31, the added nickel reagent may be derived from an aqueous nickel sulfate stock solution stored in the tank 32, the added hypophosphite reagent may be derived from an aqueous sodium hypophosphite stock solution stored in the tank 33, water may be stored in the tank 34, and an aqueous sulfuric acid stock solution may be stored in the tank 35. It will be understood that the valves 41, 42, 43 and 44 are appropriately manipulated in order to bring about the required addition of the reagents from the tanks 31, 32, 33 and 34 into the regeneration compartment 20a, while the valves 51, 52, 53 and 54 are appropriately manipulated in order to bring about the required addition of the reagents from the tanks 31, 32, 33 and 34 into the regeneration compartment 20b.

Finally, the system comprises apparatus 60 that is employed, as explained more fully hereinafter, for the removal of phosphite and other ions, the inlet to the apparatus 60 being selectively connected to the lower portion of the secondary vacuum flash tank 15 via an associated control valve 61, and the outlet from the apparatus 60 being selectively connected to the regeneration compartments 20a and 20b via respective control valves 62a and 62b.

As a matter of operating procedure, the plating solution may be continuously circulated from one of the reservoirs (for example, the reservoir 11a) to the plating tank 21 and back to the one reservoir 11a; and the plating solution may be continuously regenerated in the regeneration compartment 20a by the continuous addition of the reagents thereto by proper manipulation of the control valves 41, 42, 43 and 44. Of course, this regeneration of the plating solution only restores the composition thereof with respect to nickel cations, hypophosphite anions and pH, but does not restore the initial composition thereof with respect to the ions that are built-up therein, both by the plating reactions and by the additions of the reagents mentioned. In other words, as the plating solution is used in the plating operation, phosphite anions build-up therein, and likewise in the supply of make-up reagents thereto both sodium cations and sulfate anions are built-up therein (assuming that the stock solutions employed comprise nickel sulfate and sodium hypophosphite, as previously mentioned).

Accordingly, after predetermined utilization of the plating

solution in the continuous plating system and continuous regeneration thereof with respect to the supply of make-up reagents thereto, it is necessary to effect a regeneration of the plating solution by the utilization of the apparatus 60 so as to bring about the removal from the plating solution of the phosphite anions, as well as the sodium cations and the sulfate anions. At this time, the control valve 23a is closed and the control valves 61 and 62b are opened, and operation of the apparatus 60 is initiated, as explained more fully hereinafter; whereby the plating solution from the lower portion of the secondary vacuum flash tank 15 is circulated through the apparatus 60 and thence into the regeneration compartment 20b of the reservoir 11b. At this time, the control valves 52, 53, 54 and 55 are appropriately controlled in order to cause the supply of the required make-up reagents into the regeneration compartment 20b so as substantially completely to restore the initial composition of the chemical plating solution. In order to accommodate the complete removal of the depleted plating solution from the reservoir 11a, the control valve 22a is opened to place the lower portion of the reservoir 11a into communication with the inlet of the pump 18.

In view of the foregoing, it will be understood that the depleted plating solution is circulated from the reservoir 11a through the plating tank 12 and thence into the apparatus 60 and then into the reservoir 11b. Subsequently the restored plating solution is circulated from the reservoir 11b through the plating tank 12 and thence back into the regeneration compartment 20b of the reservoir 11b, the control valves 61, 23a and 22b being operated into their closed positions and the control valves 23b and 21b being operated into their open positions at this time, whereby operation of the apparatus 60 may be arrested.

In view of the foregoing description of the mode of operation of the continuous plating system, it will be understood that as the plating solution is circulated from the reservoir 11a through the plating chamber 12, it is continuously regenerated by the addition thereto of nickel cations, hypophosphite anions and hydroxyl anions, employing the make-up equipment 30; and after a predetermined utilization thereof, it becomes necessary to regenerate it by the removal therefrom of phosphite anions, sodium cations and sulfate anions, employing the apparatus 60, followed by the addition thereto of nickel cations, hypophosphite anions and hydrogen cations, employing the make-up equipment 30. This predetermined utilization and consequent depletion of the plating solution is manifest by the build-up therein of a phosphite anion concentration within the approximate range 0.7 to 1.5 m. p. l., and is normally reached when the accumulative nickel salt addition is such that about 400% to 500% nickel cations (with respect to the initial nickel cation content of the plating solution) have been added thereto in the continuous regeneration thereof, employing the make-up equipment 30.

Considering now in greater detail the matter of the removal of the phosphite anions, together with the sodium cations and the sulfate anions, from a depleted plating bath in the apparatus 60, it is first noted that the desirable values contained in the depleted plating bath are recovered and the resulting aqueous solution is reconstituted to provide the restored plating solution. Specifically, the pH of the depleted plating bath is first adjusted to 3.0 with sulfuric acid, and then an aqueous slurry of ferric sulfate is added thereto in order to bring about the conjoint precipitation of ferric phosphite and ferric hypophosphite; which composite precipitate is removed by filtration in a Filter Cake I, producing a Filtrate I containing substantially all of the nickel and sodium cations, substantially all of the sulfate and organic anions and small amounts

of the phosphite and hypophosphite anions, as illustrated in the following flow sheet:

*Flow sheet I*



To Filtrate I thus produced, there is added an aqueous slurry of barium hydroxide in order to precipitate barium sulfate; which precipitate is removed by filtration in a Filter cake II, producing a Filtrate II containing substantially all of the nickel cations, some of the sodium cations, small amounts of the phosphite and hypophosphite anions, some of the sulfate anions and substantially all of the organic anions, as illustrated in the following flow sheet:

*Flow sheet II*



Filtrate II thus produced is then cooled to a relatively low temperature, about  $0^\circ$  to  $5^\circ$  C., while bubbling therethrough a small amount of gaseous carbon dioxide throughout a time interval of about 30 minutes in order to precipitate sodium sulfate and some sodium carbonate and sodium bicarbonate; which precipitates are removed by filtration in a Filter cake III, producing a Filtrate III containing substantially all of the nickel cations, small amounts of the sodium cations, small amounts of the phosphite anions, hypophosphite anions and sulfate anions and substantially all of the organic anions, as illustrated in the following flow sheet:

*Flow sheet III*



Filtrate III thus produced is employed as the base of a restored plating solution, since it contains the desired values of nickel cations and organic anions; and specifically Filtrate III is reconstituted by the addition thereto of the required small amount of nickel sulfate and the required larger amount of sodium hypophosphite, together with required pH adjustment to the initial value of about 4.6, utilizing  $\text{H}_2\text{SO}_4$  and  $\text{NaOH}$  as required, so as to provide the restored plating bath of the required composition.

In the treatment, the pH of the depleted Bath IIIB is first adjusted to about 3.0 with sulfuric acid prior to the addition of the ferric sulfate, so as to bring about the conjoint precipitation of ferric phosphite and ferric hypophosphite. Subsequently, the excess sulfate anions are removed from Filtrate I by the reaction with barium hydroxide, precipitating barium sulfate. Ultimately, most of the sodium cations are removed from Filtrate II by the cooling and the reaction with gaseous carbon dioxide, precipitating conjointly sodium sulfate, sodium carbonate and sodium bicarbonate.

In view of the foregoing, it will be understood that in the continuous chemical nickel plating process, the effective or useful life of the initial plating solution may be greatly extended by the regeneration thereof, including the removal of the undesirable phosphite anions, sodium cations and sulfate anions therefrom, without the introduction thereto of foreign ions, whereby the plating solution may be restored any number of times after a corresponding number of intervening depletions thereof.

In the foregoing description, periodic or intermittent regeneration of the plating solution, with respect to the removal of sodium cations, phosphite anions and sulfate anions, in the continuous plating system was explained; however, it will be understood that this regeneration of the plating solution in the system may be continuous. This may be accomplished in a ready manner by opening the control valves 61 and 62a (utilizing the reservoir 11a) so that the apparatus 60 is arranged in bypassing relation with respect to the direct return of the plating solution to the regeneration compartment 20a, the control valve 23a also being open at this time. Thus in the arrangement, two portions of the plating solution from the lower portion of the secondary vacuum flash tank 15 respectively flow directly into the regeneration compartment 20a via the control valve 23a and indirectly into the regeneration compartment 20a via the control valve 61 and the apparatus 60. By treatment of the portion of the plating solution passing through the apparatus 60, in the manner previously explained, the required removal of phosphite anions, sodium cations and sulfate anions may be accomplished upon a continuous basis so as to prevent excessive depletion thereof in the continuous plating operation.

Accordingly, it will be understood that there has been provided a continuous chemical nickel plating process that is highly suitable for use on an industrial scale, that involves regeneration of the plating bath, as it becomes depleted with use, in a simple manner, thereby rendering the plating bath of exceedingly long life and contributing to overall efficiency of the continuous chemical nickel plating process.

While there has been described what is at present considered to be the preferred embodiment of the invention, it will be understood that various modifications may be made therein, and it is intended to cover in the appended claims all such modifications as fall within the true spirit and scope of the invention.

What is claimed is:

1. The continuous process of chemically plating with nickel a body essentially comprising an element selected from the group consisting of iron, cobalt, nickel, aluminum, copper, silver, gold, palladium and platinum; which comprises providing an aqueous plating solution of the nickel cation-hypophosphite anion type and having an initial composition including a pH in a first given range from about 4 to about 7 and a nickel cation concentration in a second given range and a hypophosphite anion concentration in a third given range; holding a portion of said solution in a plating chamber at a plating temperature disposed below the boiling point thereof but well above room temperature; immersing said body in the portion of said solution in said plating chamber to effect nickel plating on the surface thereof; withdrawing said

body from the portion of said solution in said plating chamber after a time interval corresponding to the thickness of the nickel plating on the surface of said body that is desired; said nickel plating of said body resulting from the reduction of nickel cations to metallic nickel with the corresponding oxidation of hypophosphite anions to phosphite anions, whereby during said time interval both nickel cations and hypophosphite anions are depleted and both hydrogen cations and phosphite anions are produced in the portion of said solution in said plating chamber, with the result that the portion of said solution in said plating chamber tends to depart substantially from said initial composition; withdrawing during said time interval a part of said solution from said plating chamber; treating during said time interval the withdrawn part of said solution to restore the same substantially to said initial composition; said treatment of the withdrawn part of said solution including removing therefrom by precipitation as ferric hypophosphite a major fraction of the contained hypophosphite anions and removing therefrom by precipitation as ferric phosphite a major fraction of the contained phosphite anions, without removing therefrom any more than a minor fraction of the contained nickel cations and without introducing thereinto any substantial foreign ions, followed by adding thereto sufficient hydroxyl anions to restore the pH thereof into said first range and sufficient nickel cations to restore the concentration thereof into said second range and sufficient hypophosphite anions to restore the concentration thereof into said third range; and returning during said time interval a portion of the restored part of said solution into said plating chamber.

2. The process of regenerating a depleted aqueous chemical nickel plating solution containing substantial nickel cations and substantial hypophosphite anions and considerable phosphite anions and a given organic additive to produce a restored aqueous chemical nickel plating solution containing predetermined nickel cations and predetermined hypophosphite anions and only some phosphite anions and substantially said given organic additive and having a given pH within the approximate range 4 to 7, which comprises removing from said depleted solution by precipitation as ferric hypophosphite a major fraction of the contained hypophosphite anions and removing from said depleted solution by precipitation as ferric phosphite a major fraction of the contained phosphite anions, without removing therefrom any more than a minor fraction of the contained nickel cations or any more than a minor fraction of the contained organic additive and without introducing thereinto any substantial foreign ions, whereby the resulting solution contains only some hypophosphite anions and some phosphite anions and substantial nickel cations and substantially said given organic additive, and adding to the resulting solution sufficient nickel cations to obtain said predetermined nickel cations therein and sufficient hypophosphite anions to obtain said predetermined hypophosphite anions therein and sufficient pH control ions to obtain said given pH thereof.

3. The process of regenerating a depleted aqueous chemical nickel plating solution containing substantial nickel cations and substantial hypophosphite anions and considerable phosphite anions to produce a restored aqueous chemical nickel plating solution containing predetermined nickel cations and predetermined hypophosphite anions and only some phosphite anions and having a given pH, which comprises adjusting the pH of said depleted solution to a value at least as low as 3, reacting the resulting solution with ferric sulfate to precipitate both ferric hypophosphite and ferric phosphite therein, removing the precipitated ferric hypophosphite and ferric phosphite from the reacted solution, reacting the then resulting solution with barium hydroxide to precipitate barium sulfate therein, removing the precipitated barium sulfate from the then resulting solution, and then separating the precipitated barium sulfate from the then resulting solution.

sulfate from the reacted solution, and adding to the then resulting solution sufficient soluble nickel salt to obtain said predetermined nickel cations therein and sufficient soluble hypophosphite to obtain said predetermined hypophosphite anions therein and sufficient pH control ions to obtain said given pH thereof.

4. The process of regenerating a depleted aqueous chemical nickel plating solution containing substantial nickel cations and substantial hypophosphite anions and considerable phosphite anions and some sulfate anions to produce a restored aqueous chemical nickel plating solution containing predetermined nickel cations and predetermined hypophosphite anions and only some phosphite anions and some sulfate anions and having a given pH, which comprises adjusting with sulfuric acid the pH of said depleted solution to about 3, reacting the resulting solution with ferric sulfate to precipitate both ferric hypophosphite and ferric phosphite therein, removing the precipitated ferric hypophosphite and ferric phosphite from the reacted solution, reacting the then resulting solution with barium hydroxide to precipitate barium sulfate therein, removing the precipitated barium sulfate from the reacted solution, and adding to the then resulting solution sufficient soluble nickel salt to obtain said predetermined nickel cations therein and sufficient soluble hypophosphite to obtain said predetermined hypophosphite anions therein and sufficient pH control ions to obtain said given pH thereof.

5. The process of regenerating a depleted aqueous chemical nickel plating solution containing substantial nickel cations and substantial hypophosphite anions and considerable phosphite anions and given lactic anions to produce a restored aqueous chemical nickel plating solution containing predetermined nickel cations and predetermined hypophosphite anions and only some phosphite anions and substantially said given lactic anions and having a given pH, which comprises adjusting the pH of said depleted solution to a value at least as low as 3, reacting the resulting solution with ferric sulfate to precipitate both ferric hypophosphite and ferric phosphite therein, removing the precipitated ferric hypophosphite and ferric phosphite from the reacted solution, reacting the then resulting solution with barium hydroxide to precipitate barium sulfate therein, removing the precipitated barium sulfate from the reacted solution, and adding to the then resulting solution sufficient soluble nickel salt to obtain said predetermined nickel cations therein and sufficient soluble hypophosphite to obtain said predetermined hypophosphite anions therein and sufficient pH control ions to obtain said given pH thereof, whereby said restored solution thus produced contains substantially said given lactic anions of said depleted solution.

6. The process of treating a depleted chemical nickel plating solution of the nickel cation-hypophosphite anion type to remove phosphite anions therefrom, said process comprising adjusting the pH of said depleted solution to a value at least as low as 3, reacting the resulting solution with ferric sulfate to precipitate ferric phosphite therein, and then separating the precipitated ferric phosphite from the then resulting solution.

7. The process set forth in claim 6, and further comprising reacting the then resulting solution with barium hydroxide to precipitate barium sulfate therein, and then separating the precipitated barium sulfate from the then resulting solution.

#### References Cited in the file of this patent

| UNITED STATES PATENTS |           |                               |
|-----------------------|-----------|-------------------------------|
| 70                    | 2,532,283 | Brenner ----- Dec. 5, 1950    |
|                       | 2,658,839 | Talmey ----- Nov. 10, 1953    |
|                       | 2,726,968 | Spaulding ----- Dec. 13, 1955 |